

March 4, 1958

R. B. POND

2,825,108

METALLIC FILAMENTS AND METHOD OF MAKING SAME

Filed Oct. 20, 1953

3 Sheets-Sheet 1



BY

Robert B. POND  
ATTORNEY

March 4, 1958

R. B. POND

2,825,108

METALLIC FILAMENTS AND METHOD OF MAKING SAME

Filed Oct. 20, 1953

3 Sheets-Sheet 2



INVENTOR  
ROBERT B. POND,

BY

*Robert B. Pond*

ATTORNEY

March 4, 1958

R. B. POND

2,825,108

METALLIC FILAMENTS AND METHOD OF MAKING SAME

Filed Oct. 20, 1953

3 Sheets-Sheet 3

*Fig. 5.*



*Fig. 6.*



INVENTOR

*ROBERT B. POND,*

BY

*Robert B. Pond*

ATTORNEY

## 1

2,825,108

METALLIC FILAMENTS AND METHOD OF  
MAKING SAMERobert B. Pond, Westminster, Md., assignor to Marvaland,  
Inc., Baltimore, Md., a corporation of Maryland

Application October 20, 1953, Serial No. 387,187

10 Claims. (Cl. 22—200.1)

This application relates generally to improvements in the art of metallurgy and has particular reference to a cast metallic element and the method and apparatus for making the same. This is a continuation-in-part of my application Serial No. 220,588 filed April 12, 1951, now abandoned.

More specifically, the invention deals with the transformation of molten metal into a solid product in the nature of a filament. Such a product, as produced by the method and apparatus hereinafter disclosed, may be used in almost every instance where similar products made by other methods are employed and, due to the simplicity of the method and apparatus utilized to produce the product, it is capable of being made very economically and at the point of usage. Among various commercial uses of the product are included those of thermal insulation, radio shielding, electrical resistors, special applications such as in chemical precipitation or chemical reaction tanks, ornamental tinsels; and, in military use, it provides an effective means for jamming radar reception in both offensive and defensive warfare.

Metal filaments may be divided, broadly, into two classes, the rod or wire type and the ribbon type. In both instances, the ratio of the length to the thickness of the element may be extremely large, and in the case of a ribbon filament the ratio of the length to the width may be also extremely large where the ratio between width and thickness is relatively great. Heretofore, in the production of wire type filaments, it has been the practice to draw metal wires into small diameters, and ribbon-type filaments have been produced by flat-rolling filament wires or by slitting metallic foils by various methods. These practices are known to produce plastic deformation of the metal so that, in its newly formed state, considerable residual stress, as well as a greatly distorted grain form, exists in the filament.

In accordance with the present invention, it is proposed to produce a metallic element wherein no plastic deformation is involved, with the consequence that no great residual stress exists in said element nor is there any distortion in the grain form of the metal. This desideratum is accomplished by casting the element directly from a molten material.

Extensively conducted experiments have shown that all non-refractory metals or alloys such as tin, lead, cadmium, indium, zinc, bismuth, aluminum, magnesium, copper and their alloys, and other metals and alloys of the general class specified, can be employed in making the product herein described.

It is further contemplated that the three-dimensional measurements of the elements produced may be controlled to the extent that these measurements may be made extremely small and in the order of a micron. Thus, it is possible to produce an element in the nature of a filament whose length to width ratio may be made to approach unity so that the filament becomes a particle of flake powder. Therefore, it is to be understood that the term "filament" as used in the following specification and claims is intended to include an element of powder form.

The inventive idea involved is capable of receiving a variety of expressions one of which, for purposes of illus-

## 2

tration, is shown in the accompanying drawing; but it is to be expressly understood that said drawing is employed merely to facilitate the description of the invention as a whole and not to define the limits thereof, reference being had to the appended claims for this purpose.

In the drawings:

Fig. 1 is a top plan view of an apparatus capable of carrying out the purposes of the invention;

Fig. 2 is an enlarged longitudinal section thereof taken substantially on the line 2—2 of Fig. 1;

Fig. 3 is a graph showing variation of filament thickness and length with impingement velocity;

Fig. 4 is a graph showing variation of filament thickness and length with ejection velocity;

Fig. 5 is a greatly enlarged top plan view of a piece of filament, and

Fig. 6 is a greatly enlarged bottom plan view of the same piece of filament.

The apparatus for making the product of the present invention and for carrying out the process herein disclosed consists, in its preferred form, of a base 3 upon which is mounted a chilling agent in the form of a rotary open mold chill block 4 made of a material having high conductivity and strength, whose melting temperature is above that of the metal from which the filament is formed, and which possesses sufficient mass to dissipate not only the superheat induced by raising the temperature of the metal above its melting point but also the latent heat of fusion of the filament as it is formed on the surface of the block from the stream of molten metal impinging thereon. The block is of material of great strength because of the high speeds at which the same is rotated.

Although the chill block 4 has been shown as having considerable mass, which is the desirable form of constructing the same, experiments have indicated that the open mold may take the form of a cylinder or cone also of considerable mass, or may be a continuous metallic belt upon which the molten metal impinges. Each of these latter types of mold has proven to give limited service in the production of filaments from certain of the metals hereinbefore mentioned including those having high liquid surface tension, as hereinafter referred to. However, it has been found that when the chilling agent does not possess sufficient mass to dissipate the heat of fusion of the metal being impinged upon it, there can be provided an external coolant for said agent, and this may be accomplished in any desired and well known manner.

The chill block 4, as shown, must be provided with a very smooth, polished open chill surface preferably in the form of a spherical or ellipsoidal concavity 5. The exact curvature of this surface will vary as the surface tension of the metal used to produce the filaments. By having a concave surface, the centrifugal action of the mold develops in the molten metal a higher normal force against the mold surface, thereby rupturing the surface of the metal at the point of impact and producing the intimate contact desired and its accompanying chilling effect. Thus, use is made of the centrifugal force in the metal after impingement to break down the surface tension and facilitate freezing. The higher the surface tension of the filament material at the temperature of ejection thereof toward the mold, the more difficult it is to force the stream against the mold with sufficient velocity to cause that surface or intimate contact which facilitates heat flow from the liquid stream to the chill block, and the shorter need be the radius of the concavity 5 in order to accomplish the desired chilling effect; and thus it is contemplated that the curvature of the mold surface may be changed to meet varying conditions. This type of surface has the advantage of varying surface velocity as the impingement point is varied, in a manner

to presently appear, from the center to the outer periphery of the surface.

The chill block 4 is driven about its vertical axis of rotation by means of a high speed motor 6 suitably mounted on the base 3. It is desirable that the speed of the motor may be varied to cover a rather wide range as it has been found that speeds of from approximately ten to thirty thousand R. P. M. have produced efficient results. In any event, it is essential that the surface speed of the chill block at the point of impingement of the molten metal be sufficiently high to cause the metal, solidified by contact with the surface 5 as a result of removal of the latent heat of fusion from the liquid, to be rapidly cast off by centrifugal force generated by the rotating block.

It has been stated that the chill block 4 should be provided with a very smooth polished surface 5. The smoothness should be such that there are no reentrant or sharp angles or surface changes more than those of the thickness within the width of the filament being produced.

Finishes have been effected on the chill block of from less than 1 microinch to approximately .001 inch, as checked with a profilometer. A coarse finish can only be used on heavy filaments and even then it has been found difficult to have the equipment operate well in a continuous manner. Thin filaments have been produced on a surface finish of from less than 1 microinch to approximately 40 microinches. Roughly speaking, the surface finish cannot be coarser than the thickness of the filament to be produced.

A continuous flow of molten metal to the surface 5 may be accomplished in various ways and, as shown herein, this result is attained by employing an open-ended container or ejector tube 7 provided at one end with a nozzle 8 having a restricted orifice 9 whose size may be regulated in any suitable manner such as by removably mounting said nozzle so that it can be replaced by another one having an orifice of different dimension. The opposite end of the container formed by the apertured head 10 is designed to receive, through its inlet, pressure which may be mechanically or pneumatically generated. For this purpose, said head 10 has connected thereto a pressure inlet pipe 11 adapted for connection to any suitable source of pressure supply (not shown) capable of varying said pressure to eject the molten metal through the orifice 9 in a stream and onto the revolving surface 5 with a velocity that will force said metal to make such intimate contact with said surface that heat will flow from said metal to thus produce solidification thereof. The molten metal, the temperature of which may be varied in accordance with the particular metal used and which may be increased above the melting point of the metal in order to increase its fluidity, is supplied to the container 7 from a reservoir 12 mounted thereon and from which the flow into the container may be regulated by a valve 13 in the outlet of the reservoir.

The container 7, whose nozzle 9 is disposed in proximity to the surface 5 so that the point of impingement will coincide with a radius of said surface, is carried at an incline by a wide support 14 on the base 3, and a dovetail connection 15 between said support and container enables the latter to be slidingly adjusted to vary said point of impingement of the molten metal along a line coincident with said radius or, in other words, to different positions between the center of rotation of the block 4 and the periphery of its surface. The purpose of providing this variable will become apparent as the description proceeds. It will be understood, of course, that the materials of which the container 7, its nozzle, the reservoir 12 and associated parts are made, must necessarily be such that they will not readily alloy with the molten metals since this would result in deterioration of the apparatus.

It is now apparent that the metal is ejected from the

container 7 as a liquid stream and impinges on the open surface 5 of the chill block 4 as a liquid, and that the superheat and the latent heat of fusion is removed from the liquid by intimate contact with said block, and is thus solidified and thrown from the surface 5 by the centrifugal force produced by rotation of the block. Therefore, continuity exists between the molten metal in the container 7, the molten metal in the air on its course to the surface 5, and the liquid and solid metal on said surface; and also between the solid metal on said block and that which has already left the block provided, of course, that the variables hereinafter described are controlled so as to produce a continuous filament which latter effect can be produced by a constant maintenance of supply of molten metal in the container 7.

The variables (1) temperature of the molten metal, (2) velocity of ejection from the container 7, and (3) the size of the orifice 9 can be correlated with (4) the surface speed produced by the rotating block 4 at the point of impingement of the molten metal to cast filaments of various thicknesses, widths and lengths; and, by altering one or more of said variables during the casting process, actual variations in said dimensions may be accomplished.

Generally speaking, it can be stated that the higher the temperature of the molten metal and the slower the ejection velocity thereof, with a given orifice size and mold surface speed, the thinner the filaments. Also, with all other variables held constant, the closer the velocity of ejection approaches that of surface speed at the point of impingement, the greater the continuity of the produced filament. Further, with all other variables held constant, the larger the orifice size, the wider the filament.

The formulae for these controls may be more specifically explained as follows. If the surface speed of the chill block at the point of impingement is fixed, and the impingement point is held at some constant distance from the center of rotation with the orifice size fixed, the length as well as the width of the filament or filaments is fixed. However, there are still available two other variables, namely, the temperature of the molten metal and its ejection velocity. If it be assumed that the temperature is held constant and the ejection velocity is varied, an increase in the latter will effect a tendency on the part of the molten metal to pile up on the chill block with the result that the filament will increase in thickness. Conversely, as said ejection velocity is decreased, said pile-up is lessened until, at a given velocity, the thinnest continuous filament possible will be produced with the given working temperature of the molten metal; and further reduction in said velocity will result in discontinuous filaments. Progressive reduction in the ejection velocity will produce shorter and shorter filaments until, as previously suggested, the length to width ratio of the filament approaches unity and the filament becomes a particle of flake powder.

In the event that a variation in the thickness of the filament is desired without altering the ejection velocity, the method of control can be found in the temperature of the molten metal. If this temperature is increased, the fluidity of the metal is increased or, in other words, the surface tension of the metal is decreased and a greater energy is imparted to the metal. This excess energy must be absorbed before the metal solidifies or, otherwise, during the period of contact with the chill block the metal will be in a liquid form for a longer period of time. If the ejection speed is such as to produce discontinuous filaments at one temperature, then at a higher temperature the filament will become continuous although the amount of metal ejected per unit of time is the same, and a thinner filament will be the result. Thus, in order to produce the thinnest filament possible, an exceedingly high molten metal temperature is used with some minimum ejection velocity relative to

some exceedingly high surface speed at the point of impingement.

Assuming now that the temperature, speed of ejection, orifice size, and speed of rotation of the chill block are all maintained constant, it is possible under these conditions to alter the effective surface speed at the point of impingement by translating this point between a position slightly offset from the axial center of the block and a position adjacent the peripheral edge thereof. It may be assumed that, with the above constants, the thinnest continuous filament is produced with the impingement point located halfway between said limits. Under this assumption, adjustment of the container 7 with its nozzle 8, in the manner heretofore described, toward the center of rotation of the block 4 will continue to produce an endless filament but it will become progressively thicker and, conversely, translation of the nozzle toward the periphery of the block will produce discontinuous filaments of decreasing lengths until the above mentioned powder material is attained. It should also be noted that a long continuous filament can be produced which has a varying thickness, by moving the point of impingement slowly toward the center of the mold surface while said filament is being formed.

If the angle of incidence which the stream of molten metal forms with the surface of the chill block is varied, no apparent effect upon the filament is observed. However, the angle of incidence with which the solid metal leaves the surface is a function of the continuity of filament, the thickness and width thereof or mass per unit length, the density of the metal used, the degree of polish of the surface 5 and the surface speed of the chill block at the point of impingement. Thus, the angle of incidence of the departing solid metal can be fixed relative to some external instrumentality such as a collecting bin or the like since the point of departure is dependent upon the point at which the molten metal impinges relative to said instrumentality. Hence, with the trajectory of the filament fixed, it is possible to aim the departing filament in a given direction.

Fig. 3 is a graph showing the variation of length and thickness with the parameter of impingement velocities. Fig. 4 is a similar graph showing the variation of length and thickness with the parameter of ejection velocities.

With respect to Fig. 3, as the ejection velocity is maintained at about 150 feet per second (orifice size, temperature of metal and type of metal or alloy being constant), there will be continuous filaments (ranging in thickness from 1000 microns down to just above zero) as the impingement velocity is increased from, say 50 to 400 feet per second. Thereafter, there will be discontinuous filaments with a progressive decrease in length until a flake powder stage is reached well before an impingement velocity of 1000 feet per second is reached.

As seen in Fig. 4, with an impingement velocity maintained at 600 feet per second (and with orifice size, temperature of metal and type of metal or alloy being constant), there will be a flake powder with ejection velocities ranging from 0 to a little over 200 feet per second. Discontinuous filaments will be evident before 300 and these increase in length until, when the ejection velocity reaches about 600 feet per second, continuous filaments result.

The minimum thickness figure indicated by the dark lines in Figs. 3 and 4 is 1.0 micron. These graphs, Figs. 3 and 4, show "tendency" curves. It will be appreciated that the shape of the curves and their positions relative to the abscissa and ordinate will vary as the metal or alloy is varied, or as the orifice size, or temperature of the specific metal changes, or as the relative ejection and impingement velocities change. The figures do, however, illustrate the extent of control possible. The precision of control is, of course, no better than the precision of control of all the variables.

By using a chill block such as described with surface impingement speeds varying from slightly above zero to one thousand feet per second, filaments have been produced whose minimum dimensions range from approximately 1.8 to 4.0 microns in width and thickness, and as long as two thousand feet. Under ideal conditions filaments having a minimum thickness of 1 micron and a minimum width of 1 micron can be produced.

It should be further noted that with the production of a given thickness of filament, the heat which must be absorbed by the chill block per unit of time increases as the width of the filament increases so that with unusually wide filaments it is necessary to provide an external coolant for the chill block, or otherwise the length of the filament produced during any one run of metal is limited.

In actual experiments, the greatest thickness and width so far produced in a continuous filament are a 100-microns thickness and a 5000-microns width. The greatest thickness and width so far produced in discontinuous filaments are a 700-microns thickness and a 6000-microns width. It should here be noted that the discontinuity of the filament is not due to the difference in ejection and impingement velocities but rather to the limited heat capacity of the chill block.

Although these minimum and maximum measurements may be considered as ranges for all practical purposes, it is not to be understood that the invention is, in any sense, to be limited to such ranges. Actually, it should be possible, with a continuing supply of molten metal, to extend the length of a filament to infinity.

As previously pointed out, the type of impingement surface herein illustrated has the advantage of varying surface velocity as the impingement point is varied from the center of rotation to the periphery of the surface. This would also be true of the surface of a cone, for as the point of impingement is translated parallel to the axis of symmetry of the cone the surface velocity is changed. However, since the cone has a convex surface, the only method of handling the changing surface tension problem is by altering the temperature of the molten charge.

Mention has been made herein of the fact that the filaments produced in accordance with this invention are cast metal filaments. It should now be apparent also that these cast metal filaments are solidified in a rectilinear shape with only one mold wall, namely, the smooth polished open surface of the chill block. Actually, the top and bottom surfaces of the cast metal ribbon-type filaments formed are separately and clearly identifiable, only the bottom surface bearing any indications of having engaged a mold surface. Greatly enlarged views of the top and bottom surfaces of such a filament are shown respectively in Figs. 5 and 6.

With regard to Fig. 5 it may be helpful in understanding this figure if reference is made to a technical paper, TP 3159 E, Journal of Metals, December 1951, Transactions AIME. It is clear from the two figures however that the upper surface is characterized by shrinkage marks, relief dendrites, and line striae or mammiforms, whereas the bottom surface (Fig. 6) which has engaged the chill block is smooth with the exception of polishing pit marks, buffing marks, and the imprint caused by any engraving or the like on the block.

A cast metal filament may be readily distinguished from filaments formed by other processes, as, for example, a cold wrought or cold wrought and annealed filament, by virtue of differences existing in the microstructural characteristics of the filaments. A cast filament has non-uniform large grains of non-uniform shape whereas wrought filaments have grains which are uniformly small and of uniform shape. Furthermore, the cast filament microstructure consists of heterogeneous phase or inclusion distribution in contradistinction to filaments formed by other methods. The sub-grain structure of the cast

filament is mosaic compared with the polygonized sub-grain structure of wrought and annealed filaments.

In accordance with the invention cast metal filaments have been produced where the solidification has been effected at rates of from 50 to 1000 feet per second. As will be appreciated from the foregoing description these rates may be controllably varied to effect various desired results.

In view of the great speed of solidification effected it is pertinent to note the method of measuring the solidification rate. The cast filaments formed carry on their bottom surfaces the impression of any mark placed on the chill surface. Since the surface tension of all molten metals is high it is obvious that the metal must have solidified while on the chill surface. The metal is never on the chill surface for one complete revolution of the surface (for if it was it would result in overlay or piling up of the material). In fact, with the present invention as described, only about one-half inch of the filament contacts the surface at any one time, that is to say, the molten metal goes onto the surface of the chill block at the same rate that the solid cast metal comes off. Then, since it is transformed from a liquid to a solid while on the rotating chill block, its minimum velocity of solidification can be calculated knowing the speed of the surface at the point of impingement and the length of filament making contact at any one time.

So that the invention will be more clearly understood, the following specific examples are given:

#### EXAMPLE 1

Employing an aluminum chill block having a diameter

of 3", a weight of .6 lb. and a radius of curvature of 5", and having a surface finish of 30 microinches; and employing a glass round orifice having a diameter of 30 $\mu$ ; molten tin having a surface tension of 526 dynes per cm. at  $\Delta Ts=50$ , was ejected at 75 ft./sec. at a pressure of 6 lbs. The velocity of impingement was 300 ft./sec. and the angle of impingement was 90°. Filaments were produced having a length of 15 feet, a thickness of 10 $\mu$  and a width of 200 $\mu$ .

5 Note.—The symbol  $\Delta Ts=50$  signifies that the temperature of the metal at ejection was the melting temperature plus 50°.  $\mu$  signifies microns.

#### EXAMPLE 2

With the same chill block, orifice, and metal as in Example 1, but employing a velocity of ejection of 300 ft./sec. at a pressure of 15 lbs., and an angle of impingement of 10°, filaments were produced having a length of 22 feet, a thickness of 27 $\mu$  and a width of 300 $\mu$ .

#### EXAMPLE 3

15 In this example, a chill block similar to Example 1 was employed, but with a finish of 2 microinches. The orifice used was of silicon carbide. Tin having a surface tension of 514 dynes per cm. at  $\Delta Ts=200$  was ejected at a velocity of 75 ft./sec. at a pressure of 6 lbs. The velocity of impingement was 300 ft./sec. and the angle of impingement was 60°. Filaments were produced having a length of 75 feet, a thickness of 6.5 $\mu$  and a width of 220 $\mu$ .

20 25 30 These and other examples of tin are listed in the following tabulations:

| Chill Block |    |      |     |    | Orifice |     |           | Metal       |       | Ejection     |    | Impingement  |     | Filament  |             |           |
|-------------|----|------|-----|----|---------|-----|-----------|-------------|-------|--------------|----|--------------|-----|-----------|-------------|-----------|
| M.          | D. | Wt.  | CR. | F. | M.      | Sh. | D.        | $\Delta Ts$ | S. T. | V.           | P. | V.           | A.  | T.        | W.          | L.        |
| Al          | 3" | .6#  | 5   | 30 | Glass   | O   | 30 $\mu$  | 50          | 526   | 75 ft./sec.  | 6  | 300 ft./sec. | 90° | 10 $\mu$  | 200 $\mu$   | 15 ft.    |
| Al          | 3" | .6#  | 5   | 30 | Glass   | O   | --        | 50          | 526   | 300 ft./sec. | 15 | 300 ft./sec. | 10° | 27 $\mu$  | 300 $\mu$   | 22 ft.    |
| Al          | 3" | .6#  | 5   | 2  | SIC     | O   | --        | 200         | 514   | 75 ft./sec.  | 6  | 300 ft./sec. | 60° | 6.5 $\mu$ | 220 $\mu$   | 75 ft. <  |
| Steel       | 7" | 2.4# | 10  | 50 | Steel   | O   | 300 $\mu$ | 60          | 526   | 300 ft./sec. | 15 | 300 ft./sec. | 10° | 8 $\mu$   | 230 $\mu$   | 100 ft. > |
| Steel       | 7" | 2.4# | 10  | 50 | Steel   | O   | 300 $\mu$ | 60          | 526   | 75 ft./sec.  | 4  | 300 ft./sec. | 30° | 18 $\mu$  | 2,000 $\mu$ | 10 ft.    |

#### Legend:

M.—Material.

D.—Diameter.

Wt.—Weight.

CR.—Radius of curvature in inches.

F.—Finish in micro-inches.

Sh.—Shape—round.

$\Delta Ts$ —See note above.

S. T.—Surface tension in dynes/cm.

V.—An approximation of ejection velocity.

P.—Pressure in pounds.

Vi.—Impingement velocity.

A.—Angle.

T.—Thickness.

W.—Width.

L.—Length.

Examples employing zinc as the filament metal are as follows:

| Chill Block |    |     |     |    | Orifice |     |          | Metal       |       | Ejection    |    | Impingement  |     | Filament |           |          |
|-------------|----|-----|-----|----|---------|-----|----------|-------------|-------|-------------|----|--------------|-----|----------|-----------|----------|
| M.          | D. | Wt. | CR. | F. | M.      | Sh. | D.       | $\Delta Ts$ | S. T. | V.          | P. | V.           | A.  | T.       | W.        | L.       |
| Al          | 3" | .6# | 5   | 2  | Glass   | O   | 30 $\mu$ | 100         | 778   | 75 ft./sec. | 8  | 300 ft./sec. | 30° | 15 $\mu$ | 300 $\mu$ | 2 ft.    |
| Al          | 3" | .6# | 5   | 2  | SIC     | O   | 30 $\mu$ | 100         | 778   | 75 ft./sec. | 8  | 500 ft./sec. | 30° | 15 $\mu$ | 180 $\mu$ | 4 in.    |
| Al          | 3" | .6# | 5   | 2  | Mo.     | O   | 30 $\mu$ | 100         | 778   | 75 ft./sec. | 8  | 800 ft./sec. | 30° | 15 $\mu$ | 50 $\mu$  | 70 $\mu$ |

Examples employing lead as a filament metal are as follows:

| Chill Block |    |      |     |    | Orifice |     |          | Metal       |       | Ejection     |    | Impingement  |     | Filament |           |           |
|-------------|----|------|-----|----|---------|-----|----------|-------------|-------|--------------|----|--------------|-----|----------|-----------|-----------|
| M.          | D. | Wt.  | CR. | F. | M.      | Sh. | D.       | $\Delta Ts$ | S. T. | V.           | P. | V.           | A.  | T.       | W.        | L.        |
| Steel       | 7" | 2.4# | 10  | 50 | Steel   | O   | 30 $\mu$ | 100         | 438   | 140 ft./sec. | 9  | 200 ft./sec. | 30° | 9 $\mu$  | 480 $\mu$ | 75 ft. <  |
| Al          | 3" | .6#  | 5   | 2  | Steel   | O   | 30 $\mu$ | 100         | 438   | 140 ft./sec. | 9  | 200 ft./sec. | 30° | 4 $\mu$  | 590 $\mu$ | 100 ft. > |
| Steel       | 7" | 2.4# | 10  | 50 | Steel   | O   | 14 $\mu$ | 100         | 438   | 140 ft./sec. | 9  | 200 ft./sec. | 30° | 7 $\mu$  | 160 $\mu$ | 100 ft. > |

Examples employing a brass as the filament metal are:

| Chill Block |    |      |     |    | Orifice |     |          | Metal       |       | Ejection     |    | Impingement    |     | Filament |           |          |
|-------------|----|------|-----|----|---------|-----|----------|-------------|-------|--------------|----|----------------|-----|----------|-----------|----------|
| M.          | D. | Wt.  | CR. | F. | M.      | Sh. | D.       | $\Delta Ts$ | S. T. | V.           | P. | Vl.            | A.  | T.       | W.        | L.       |
| Brass       | 4" | 1.3# | 5   | 2  | SiC     | O   | 30 $\mu$ | 50<         | ---   | 25 ft./sec.  | 3  | 1,000 ft./sec. | 30° | 3 $\mu$  | 6 $\mu$   | 8 $\mu$  |
| Brass       | 4" | 1.3# | 5   | 2  | SiC     | O   | 30 $\mu$ | 50>         | ---   | 75 ft./sec.  | 12 | 1,000 ft./sec. | 30° | 3 $\mu$  | 48 $\mu$  | 75 ft.>  |
| Brass       | 4" | 1.3# | 5   | 2  | SiC     | O   | 30 $\mu$ | 50<         | ---   | 150 ft./sec. | 25 | 1,000 ft./sec. | 30° | 3 $\mu$  | 180 $\mu$ | 100 ft.> |

Examples employing copper as the filament metal are:

| Chill Block |     |      |     |    | Orifice |     |           | Metal       |       | Ejection     |    | Impingement  |     | Filament  |             |          |
|-------------|-----|------|-----|----|---------|-----|-----------|-------------|-------|--------------|----|--------------|-----|-----------|-------------|----------|
| M.          | D.  | Wt.  | CR. | F. | M.      | Sh. | D.        | $\Delta Ts$ | S. T. | V.           | P. | Vl.          | A.  | T.        | W.          | L.       |
| Steel       | 7"  | 2.4# | 10  | 50 | SiC     | O   | 3 $\mu$   | 60          | ---   | 100 ft./sec. | 60 | 400 ft./sec. | 30° | 9 $\mu$   | 13 $\mu$    | 6 $\mu$  |
| Steel       | --- | ---  | 10  | 50 | SiC     | O   | 30 $\mu$  | 50          | ---   | 100 ft./sec. | 30 | 400 ft./sec. | 30° | 19 $\mu$  | 76 $\mu$    | 18 ft.   |
| Steel       | --  | --   | 10  | 50 | SiC     | O   | 300 $\mu$ | 50          | ---   | 100 ft./sec. | 3  | 50 ft./sec.  | 30° | 100 $\mu$ | 1,200 $\mu$ | 100 ft.> |

The invention has also been used to make filaments of cadmium, bismuth, indium, magnesium, aluminum and various alloys of these. Among the alloys tried have been Pb-Sn 32-68, 50-50, 60-40; Zn-Sn 50-50; Cu-Zn 70-30, 90-10; Al-Si 97-3; Al-Cu 97-3. (The numbers after the metals indicate the percentages in order.)

An example of the effect of a change in the radius of curvature of the chill block is of interest.

An aluminum chill block having a radius of curvature of 10" was used. A round orifice of a diameter of .010" was employed with an ejection velocity of 75 F. P. S. and an impingement velocity of 200 F. P. S. Employing tin having a surface tension of 522 dynes per cm. at  $\Delta Ts=100$ , filaments were formed. But, employing zinc having a surface tension of 778 dynes per cm. at  $\Delta Ts=100$ , no filaments would form. However, with everything else held constant, the radius of curvature of the chill block was changed to 5 inches and both tin and zinc then formed filaments.

It should be noted that aluminum cannot be formed into a filament on a chill block having a 10" radius of curvature regardless of the  $\Delta Ts$ . Moreover, if no concavity at all is used, and the ejection velocity is kept low, no filament will be produced but instead, the metal will roll off the edge of the chill block in the form of little balls.

In accordance with the invention it is possible to produce a plurality of filaments simultaneously and with the same apparatus. To effect this a plurality of spaced nozzles or spaced orifices may be employed. Other variations of the invention will occur to those skilled in the art who have knowledge of this disclosure.

I claim:

1. A new article of manufacture comprising, a cast metal filament the thickness of which ranges from approximately 1 to 4 microns, and the length of which ranges from approximately 1 micron to infinity.

2. A new article of manufacture comprising, a cast metal filament the width of which ranges from approximately 1 to 4 microns and the length of which ranges from approximately 1 micron to infinity.

3. A new article of manufacture comprising a cast metal filament the thickness and width of which range from approximately 1 to 4 microns, and the length of which ranges from approximately 1 micron to infinity.

4. A new article of manufacture comprising a cast metal filament having mold marks on one surface only, said filament having a thickness which ranges from 1 to 4 microns, said filament having a relatively great width to thickness ratio and a length which ranges from approximately 1 micron to infinity.

25 metal filament, said filament having mold marks on one surface only and having non-uniform, comparatively large grains with a microstructure of heterogeneous phase distribution, said filament having a width which ranges from approximately 1 to 4 microns, said filament having a relatively great width to thickness ratio and a length which ranges from approximately 1 micron to infinity.

6. A method of casting solid metal filaments from molten metal which comprises impinging a stream of molten metal against a smooth polished concave open 35 chill surface, rotating said surface, the solidification of the metal being effected at a rate ranging from approximately 50 to 1000 feet per second.

7. A method of casting solid metal filaments from molten metal which comprises impinging a stream of molten metal against a smooth polished open rotatable 40 chill surface in which the plane of the surface forms an acute angle with the axis of rotation of the surface on that side of the surface on which the metal is impinged, rotating said surface, the solidification of the metal being effected at a rate ranging from approximately 50 to 1000 feet per second.

8. A method of casting solid metal filaments from molten metal which comprises impinging a stream of molten metal against a smooth polished open rotatable 50 chill surface in which the plane of the surface forms an acute angle with the axis of rotation of the surface on that side of the surface on which the metal is impinged, and rotating said surface whereby a component of the force acquired by the metal is normal to the plane of 55 the surface tending to retain the metal on the surface and solidifying the molten metal while the metal is retained on the surface.

9. The method of casting molten non-refractory metal 60 into continuous strips in widths ranging approximately from 1.8 to 5000 microns and in thickness ranging from 4.0 microns to 100 microns, which comprises impinging a stream of molten metal against a smooth polished open chill surface, rotating said chill surface, controlling the speeds of impingement and of rotation so that the metal 65 remains on the chill surface for a period less than required for one revolution, the temperature of the molten metal, the surface tension of the metal being chosen with respect to said speeds to effect solidification of the metal while on the chill surface at rates ranging from approximately 50 to 1000 feet per second.

10. The method of casting solid metal filaments from molten metal which comprises impinging a stream of molten metal against a smooth polished open chill surface, rotating said surface, and varying the point of impingement of the stream to positions between the center 75

11

of rotation and the periphery of the surface in order to vary the length and thickness of the filament, the solidification of the metal being effected at rates ranging from approximately 50 to 1000 feet per second.

## References Cited in the file of this patent

## UNITED STATES PATENTS

Re. 12,568 Cowing ----- Nov. 27, 1906  
745,786 Cole ----- Dec. 1, 1903

12

|             |                      |               |
|-------------|----------------------|---------------|
| 905,758     | Strange et al. ----- | Dec. 1, 1908  |
| 989,075     | Staples -----        | Apr. 11, 1911 |
| 1,063,895   | Staples -----        | June 3, 1913  |
| 1,291,603   | Nagy -----           | Jan. 14, 1919 |
| 5 1,695,041 | Elmen -----          | Dec. 11, 1928 |
| 2,062,093   | Kann -----           | Nov. 24, 1936 |
| 2,598,344   | Brennan -----        | May 27, 1952  |
| 2,639,490   | Brennan -----        | May 26, 1953  |
| 2,701,901   | Pawlak -----         | Feb. 15, 1955 |

UNITED STATES PATENT OFFICE  
CERTIFICATE OF CORRECTION

Patent No. 2,825,108

March 4, 1958

Robert B. Pond

It is hereby certified that error appears in the above numbered patent requiring correction and that the said Letters Patent should read as corrected below.

In the grant, lines 2 and 12, and in the heading to the printed specification, lines 4 and 5, name of assignee, for "Marvaland, Inc." read -- Marvalaud, Inc. --, in each occurrence.

Signed and sealed this 21st day of October 1958.

(SEAL)

Attest:

KARL H. AXLINE

Attesting Officer

ROBERT C. WATSON  
Commissioner of Patents